

## UNITED STATES PATENT OFFICE

2,272,277

## PROCESS OF MANUFACTURING STEEL

Edwin L. Ramsey and Leslie G. Graper,  
Chicago, Ill.No Drawing. Application April 25, 1941,  
Serial No. 390,342

8 Claims. (Cl. 75—133)

This invention relates to a new steel having improved machining properties and to a process of manufacturing such a steel.

It has been the practice, to improve the machinability of steel, to add sulphur to the steel. The making of sulphur steel at the open hearth is very simple in that the stick sulphur is added to the molten metal while it is being tapped into the ladle. The difficulty that arises is in rolling the steel at the blooming mill where the ingots have a tendency to crack in the rolls due to what is called a "red short" condition. The theory back of this condition is that the sulphur added to the steel forms iron sulphide which migrates to the grain boundaries in the steel. This iron sulphide has a low melting point resulting in a condition when the steel is rolled such that it will part or crack at these grain boundaries because of the liquid condition of the iron sulphide at the rolling temperature. This condition is overcome to some extent if the steel contains a large percentage of manganese, the sulphur combining with the manganese forming manganese sulphide, thereby preventing formation of iron sulphide. The manganese sulphide remains in the steel in globular inclusions which do not migrate to the grain boundaries resulting in a lesser formation of iron sulphide.

It has been observed that sulphur steels made by the Bessemer process, which process consists of burning the carbon out of the steel by passing air through the molten metal, does not develop a "red short" condition to the same extent as steel made in the open hearth. In this process a large quantity of oxygen passes through the steel which probably results in the formation of a different compound from iron sulphide; hence, resulting in a steel not as "red short." It has also been noticed that sulphur steel with a low carbon content usually rolls better than sulphur steel with a high carbon content. It is believed this is due to the fact that low carbon steels contain much more oxygen in solution than the higher carbon steels. It has also been found, when making sulphur additions to completely killed steel, that a small amount of sulphur will result in a "red short" condition when rolling. It is believed that this is due to the fact that killed steels are substantially deoxidized.

The present demand of the steel users for steels of all specifications which can be used in automatic machines and which can be machined very easily, has increased considerably, creating a problem for the open hearth in producing these sulphur bearing steels so that the steel will not

be "red short" when it is rolled. There have been various processes developed for the addition of sulphur by other means than as stick sulphur; for example, processes are known in which the sulphur is added as molybdenum sulphide and manganese sulphide.

A principal object of the present invention is to provide an improved process of manufacturing steel of improved machinability by removing 10 from the steel inclusions and conditions resulting from manufacturing processes which reduce tool life.

A more specific object is to provide an improved manufacturing process for adding sulphur in an 15 oxidized form to a killed steel such as open hearth steel.

A still more specific object is to obtain the 20 proper amount of sulphur in a steel and simultaneously improve the rolling and machining properties thereof by adding sulphur as sodium sulphite or sodium bisulphite.

Another object is to remove aluminates and 25 silicates and other inclusions which are apt to be detrimental to rolling or injurious to tool life by slagging of such constituents of the steel by adding a strong base or a composition which decomposes at the temperature of molten steel to provide a strong base prior to the pouring of the material into the ingots.

30 This invention contemplates steels having generally standard analyses or alloy steels in which the sulphur content is increased by the addition of sulphur in an oxidized form such as sodium sulphite and sodium bisulphite. Simultaneously 35 with the addition of sulphur, it is preferable to add or have present before decomposition of the sulphur compound, a strong base such as sodium oxide. In this respect the sodium sulphites are particularly suited as these chemicals when added 40 to the molten metal decompose or break down into sodium oxide and sulphur oxide. The molten metal picks up the sulphur, possibly as the oxide, while the sodium oxide is partially volatilized and partially reacts with any inclusions in the metal 45 of an acid nature, such as the silicates and aluminates, forming sodium silicates and aluminates which are very easily fluxed and thus removed from the steel. By the use of a chemical of this nature, sulphur is introduced into the steel in a 50 different form and at the same time some of the objectionable refractory inclusions such as silicates are removed. Steels made with the addition of these chemicals have been found to have improved or better physical qualities in every respect. Such steels roll much better, not exhibit-

ing "red shortness"; that is, cracks and seams which must be chipped out during conditioning of the billet for further rolling to such an extent as steel made with stick sulphur; better both as to life and as to speed of cut. It is believed that this better machining is due to the inclusions of the sulphur compounds being finely divided and evenly dispersed due to the fact that the sulphur is freed in the metal by decomposition of the sulphite. It is also believed that the extra tool life is due to the fact that any objectionable inclusions are removed. As inclusions such as silicates and aluminates are of a very refractory nature, such inclusions act to dull the tools very rapidly. Results which will be hereinafter set forth with the process of this invention indicate that better machinability is obtained with a smaller percentage of sulphur in the specification than has heretofore been obtained.

Although the process of this invention is particularly applicable to steels such as given in the examples to follow, other specifications which require a low sulphur content in order to obtain the desirable physical properties can be benefited by the addition of compounds which will break down into strong bases in the molten metal permitting a fluxing of the oxide with the inclusions and therefore easily removing them from the steel.

An example will be given of a steel manufactured by the process of this invention. The particular heat was to be made to the following specification:

|         |         |          |         |         |            |
|---------|---------|----------|---------|---------|------------|
| C       | Mn      | Phos.    | Sul     | Sil     | Grain size |
| .55-.60 | .60-.90 | .04 max. | .04-.07 | .15-.30 | Fine       |

The ladle analysis of the heat after completion was as follows:

|     |     |       |      |      |            |
|-----|-----|-------|------|------|------------|
| C   | Mn  | Phos. | Sul. | Sil. | Grain size |
| .55 | .75 | .016  | .045 | .19  | Fine       |

The sulphur addition to this heat was made by adding 350 pounds of anhydrous sodium bisulphite, also called sodium pyro sulphite, to the ladle after the manganese and silicon. The sulphur was increased from .025 residual in the bath to .045 by this addition. This amounts to an addition of .020 points of sulphur by means of the sodium bisulphite. This heat rolled very well in the blooming mill and in the merchant mill. A portion of the heat was rolled into round bars which were later machined from about  $1\frac{1}{8}$ " to 1" round, as is common practice. The bars were machined at the rate of 85 lineal feet per hour as compared to about 69 lineal feet per hour on bars of the other heats having the same ladle analysis except for the additional sulphur. It was also found that the tool life for the treated steel was approximately three times as long as for the untreated steel; that is, about nine bars per tool were turned as compared with one to three bars per tool with the untreated steel.

As another example of the practice of this method, a heat was made having the following analysis:

| C   | Mn  | Phos. | Sul. | Sil. |
|-----|-----|-------|------|------|
| .83 | .48 | .017  | .023 | .21  |

In order to check the sulphur distribution throughout an ingot when making a sodium bisulphite addition to a 26" mold, 6.6 pounds of sodium bisulphite were added to the first ingot

of this heat. The ingot weight was 9500 pounds; the sulphur recovery was about 70%. The first and second ingots were spotted and samples were taken for sulphur analysis, the second ingot being taken to give a comparison between the first ingot and the balance of the heat. The sulphur analyzed as follows:

|        | 1st ingot | 2nd ingot |
|--------|-----------|-----------|
| Top    | .035 sul. | .023 sul. |
| Center | .035 sul. | .022 sul. |
| Bottom | .035 sul. | .021 sul. |

There was practically no slag formation at the top of the second or untreated ingot. In the first ingot there was an appreciable slag formed at the top of the ingot. This resulted from the breaking up of sodium bisulphite into sodium oxide and sulphur dioxide. The sodium oxide volatilized to some extent but unites to a considerable degree with the acid reaction products of the deoxidation process utilized in killing open hearth steels. A sample of the slag formed at the top of the ingot analyzed as follows:

|                                |       |
|--------------------------------|-------|
| FeO                            | 3.24  |
| MnO                            | 5.55  |
| SiO <sub>2</sub>               | 36.14 |
| Al <sub>2</sub> O <sub>3</sub> | 28.77 |
| Lime                           | Nil   |
| Sul                            | 1.27  |
| Na <sub>2</sub> O              | 21.15 |

This analysis shows the large percentage of silicates and aluminates which had combined with the sodium oxide provided by the decomposition of the sulphite, thus removing these inclusions from the steel.

As a comparison of physical properties, the heat first described above was compared as to physical properties with a heat having the same specification in which stick sulphur was used as a means of introducing sulphur into the steel. This comparison is as follows:

46 Heat No. 65,504 with sodium bi-sulphite

| Elastic | Tensile | Percent elongation | Percent reduction | Impact           |                  |
|---------|---------|--------------------|-------------------|------------------|------------------|
|         |         |                    |                   | Feet             | Pounds           |
| 59,930  | 107,380 | 23.0               | 44.9              | 18 $\frac{1}{4}$ | 21               |
| 59,930  | 107,630 | 23.5               | 44.9              | 17 $\frac{1}{2}$ | 17 $\frac{1}{4}$ |
| 58,920  | 107,630 | 23.0               | 44.0              | 17               | 17 $\frac{1}{4}$ |

55 Heat No. 73,843 with stick sulphur

| Elastic | Tensile | Percent elongation | Percent reduction | Impact           |                  |
|---------|---------|--------------------|-------------------|------------------|------------------|
|         |         |                    |                   | Feet             | Pounds           |
| 58,920  | 108,900 | 21.0               | 39.4              | 8                | 10 $\frac{1}{4}$ |
| 58,420  | 108,880 | 20.0               | 39.1              | 10 $\frac{1}{4}$ | 9                |
| 58,420  | 108,050 | 20.5               | 39.4              | 11               | 11               |

|        | Analysis of heats | C   | Mn  | Phos. | Sul. | Sil. |
|--------|-------------------|-----|-----|-------|------|------|
| 65,504 |                   | .55 | .75 | .016  | .045 | .19  |
| 73,843 |                   | .55 | .63 | .020  | .062 | .13  |

70 Under the microscope at 2,000 diameters the inclusions in the bisulphite heat appeared smaller and of a very irregular shape, while in the other heat they look larger and with a smoother edge.

Applicants have defined specific examples of the addition of sulphur as a sodium bisulphite to steels of a specified composition. Other bi-

sulphites of the alkali metal group have substantially the same chemical properties in so far as the practicing of this invention is concerned. In so far as the use of a sulphite or bisulphite for obtaining free sulphur dioxide at a relatively low temperature is a part of the invention, other metal sulphites may be used, it being only necessary to obtain the results of the invention that the metallic sulphite decompose at the temperature of the fused metal being treated to give off sulphur dioxide. It is to be understood that the process of the invention can be practiced simultaneously with other processes for imparting the same or other qualities to the steel. For example, certain of the advantages of the process of this invention may be gained with the simultaneous addition of free sulphur to further increase the sulphur content of the steel. It is to be understood that they contemplate the use of their process for all steels including alloys to which the process is applicable, and all modifications of the process falling within the scope of the appended claims.

What is claimed is:

1. A process of manufacturing a steel of improved machinability comprising adding to a molten mass of steel a metallic sulphite which decomposes at the temperature of said molten mass to give up a substantial proportion of the sulphur as sulphur dioxide.
2. A process of manufacturing a steel of improved machinability comprising adding to a molten mass of steel a sodium sulphite.
3. A process of manufacturing a steel of improved machinability comprising adding to a molten mass of steel sodium bisulphite.

4. A process of manufacturing a steel of improved machinability comprising adding to a molten mass of steel before cooling in an ingot mold a sodium sulphite in amounts ranging from 5 1 to 5 pounds per ton of steel.
5. A process of manufacturing a steel of improved machinability comprising adding to molten steel before cooling in an ingot mold having an initial sulphur content of .030 to .070 a sodium sulphite in amounts ranging from 10 2 to 5 pounds per ton of steel.
6. A process of manufacturing a steel of improved machinability comprising adding to the ladle during tapping from the furnace and before pouring into an ingot mold, a steel having a composition of carbon .55, manganese .75, phosphorus .016, sulphur .020, silicon .019, sodium bisulphite at the rate of approximately 3 pounds per ton thereby increasing the sulphur content from .020 to .046 whereby certain impurities as silicates and aluminates are fluxed by the decomposition of the bisulphite into sodium oxide and sulphur dioxide and rise as a slag to the surface of the metal in the ingot.
7. A process of manufacturing a steel of improved machinability comprising adding to a molten mass of steel an alkali metal sulphite.
8. A process of manufacturing a steel of improved rolling and machining properties which comprises adding to a molten mass of steel a metallic sulphite which decomposes at the temperature of the molten mass to provide widely dispersed sulphur inclusions in the hardened metal.

EDWIN L. RAMSEY.  
LESLIE G. GRAPER.